

Feb. 16, 1926.

1,573,297

E. A. BRINER ET AL

PROCESS OF DRYING PAPER

Filed Nov. 29, 1919

2 Sheets-Sheet 1



Fig. 1.

Inventors:  
E. A. Briner  
by H. J. Gould  
Elbridge Brown, Inventor, May

Attorneys

Feb. 16, 1926.

1,573,297

E. A. BRINER ET AL

PROCESS OF DRYING PAPER

Filed Nov. 29, 1919



Patented Feb. 16, 1926.

1,573,297

# UNITED STATES PATENT OFFICE.

EMIL A. BRINER, OF EAST ORANGE, NEW JERSEY, AND HENRY J. GUILD, OF BANGOR, MAINE; SAID GUILD ASSIGNOR TO EASTERN MANUFACTURING COMPANY, OF BOSTON, MASSACHUSETTS, A CORPORATION OF MASSACHUSETTS.

## PROCESS OF DRYING PAPER.

Application filed November 29, 1919. Serial No. 341,359.

*To all whom it may concern:*

Be it known that we, EMIL A. BRINER and HENRY J. GUILD, citizens of the United States, respectively residing at East Orange, 5 in the county of Essex and State of New Jersey, and at Bangor, in the county of Penobscot and State of Maine, have invented new and useful Improvements in Processes of Drying Paper, of which the following 10 is a specification.

For the intelligent understanding of this process and the apparatus adapted to carrying it out it is necessary to clearly comprehend certain general laws having to do with 15 the drying of paper and similar materials, which laws we have ascertained by careful quantitative experiments undertaken in connection with the working out of this invention. These laws, particularly in their bearing 20 upon the invention, will first be explained, and afterwards we shall point out their application to the securing of optimum results in the drying of paper.

The formation of a sheet of paper proceeds 25 from the initial entanglement of the paper-making fibers in partial water suspension as the wet stock is flowed on the wire, through the progressive establishment of intimate contact between these fibers as the 30 water is removed by natural drainage, by suction and by pressure; and finally to the drying of this web of interlaced or felted fibers into a sheet, the tenacity of which depends upon the character and relative position of the fibers and their hold upon each 35 other, and the smoothness of which depends upon the evenness with which the initially flat wet sheet dries into a flat dry sheet.

The selection of stock, beating, refining, 40 and sheet-formation,—things with which our invention is not directly concerned,—fix the character of the wet sheet and hence determine the best results—as to strength and flatness among other things—that may finally 45 be obtained if none of the possibilities are lost in drying.

The drying operation in existing paper-machines has always heretofore been carried out under well established conditions. 50 In order to insure flatness of the sheet, the initially wet web of paper traveling from the press-rolls is held firmly in contact with the successive hot drying rolls or cylinders by the tightly engaging “felt”, and it is

under relatively strong tension where it 55 passes from one drying roll to another. This condition continues from the first drying rolls to the end of the machine, where the paper is dry, and where its character and strength, in so far as drying affects it, has 60 therefore been determined. It will be seen that in such standard drying apparatus the paper is mechanically held under restraint from shrinkage and is not allowed to take up 65 its own dimensions during this drying process; and it will be shown that this has an important effect on strength, and that great improvement may be realized by departure in certain matters from this standard practice.

Top-sized papers, coated papers, and other special papers are more or less superficially wetted again by their respective subsequent treatments after the completion of the principal drying operation just noted, 75 and certain methods other than those indicated have been used or disclosed for the second drying of such papers; but these methods are concerned with what is essentially an after-treatment, and are applied at a time subsequent to the end of the phase that we have found to be by far the most responsive or susceptible in the matter of effect of drying methods on strength—as will 80 be explained.

Our experiments developed some facts of importance that were hitherto unknown, and checked or modified some conclusions which had been regarded as established or 85 generally accepted.

It was first found that paper dried in the customary manner just described, where the web is under strong constraint throughout the drying process, showed both a bursting and a tensile strength much inferior to that of a specimen of the same paper taken from just beyond the press-rolls and air-dried without resort to any strongly effective mechanical expedient to maintain flatness. On the other hand, while the specimen of paper 90 that had been dried under mechanical restraint in the standard way was flat and even, the wholly air-dried specimen was so 95 badly “cockled” as to be quite unsalable for any ordinary purpose. This substantial sacrifice of potential strength through some action occurring during the principal drying process has been, so far as we know, 100

universally accepted as a necessary evil, in view of the requirement for flatness, and it was the purpose of our investigation to determine precisely how and where the loss 5 occurred, and further to determine whether any process and apparatus could be developed whereby retention of substantially maximum strength could be rendered compatible with the production of a flat and acceptable sheet.

The general procedure in this investigation was as follows:

During a run of a known grade and weight of paper over a paper-machine of the usual 15 type, a large sample was taken off just after the press-rolls (to which the paper is fed from the Fourdrinier wire), a similar one just after passage over the first drier-roll, and other samples after each of the other 20 succeeding drier-rolls. Each of these specimens was then air-dried without any strong mechanical constraint, tests of bursting strength and tensile strength were made on the successive dry specimens, and the results 25 compared. Other runs were similarly made on various other grades of paper and the groups of results similarly compared, and plotted as in Figure 1.

These tests disclosed the unsuspected and 30 important fact that the loss of strength did not occur progressively during the entire process of constrained drying as was anticipated; on the contrary, nearly all of the detrimental action was limited to one 35 rather brief phase of the drying process. They established the following novel and valuable conclusions; that there is a first critical moisture percentage, remarkably definite for each kind of paper, to which drying 40 under strong mechanical constraint can be carried without appreciable detriment to strength; but beyond which the continuance of any form of effective strong mechanical hold upon the wet or damp web, 45 and particularly the continuance of the customary amount of tension, causes a marked progressive decrease of strength which goes on cumulatively as a result of the usual drying procedure, through what may be termed 50 the responsive or susceptible drying phase or moisture zone, and ceases again somewhat abruptly at a second critical point when the paper becomes nearly dry. This relation is shown by the aforementioned plot 55 marked Figure 1 to which further explanatory reference is made below. In a certain 60 23-roll drier with which we worked, the first critical moisture percentage was reached for most writing papers just after the 12th roll. 65 We also found that specimens of paper taken very wet after contact with only a few of the first drying cylinders behaved in greater or less degree as did those taken directly after the press-rolls, showing on air-drying a tendency to "cockle" or dry

with marked irregular local departures from flatness, which tendency could not be overcome without resort during the early part of the drying to mechanical constraint as severe as that which would have been enforced by further passage through the paper-machine driers in the customary way. On the other hand, paper which had progressed beyond a certain fairly definite point in drying on the paper-machine, responded to unconstrained further or final drying without development of cockle or other objectionable departure from flatness.

The experiments disclosed the further important fact that this fairly definite moisture percentage at which the paper could be taken off from the machine and the drying be successfully contained in the air—or otherwise without marked mechanical enforcement of flatness,—was substantially coincident with the previously mentioned remarkably definite first critical point, where the percentage of moisture marked the beginning of the phase susceptible to injury through drying under the customary stretch and mechanical hold.

These two discoveries taken concurrently showed first that if full strength is to be conserved, the progressively drying paper must be freed from mechanical restraint 95 when, or before, it has dried down to a definite critical percentage of moisture; and second that, if flat drying is to be accomplished, the paper must not be freed from such restraint until when or after it had reached substantially this same critical moisture percentage.

The practical identity of the point beyond which drying under strong constraint may not go without detriment to strength, and the point to which it must go to insure absence of cockle, is not thought to be a mere coincidence,—as subsequently explained.

We have found then that, in order to get an optimum flat paper having unimpaired strength, the initial period of drying under relatively strong constraint, such as that found on a paper-machine, must proceed to, but not beyond a critical point, definite for that paper; and that thereafter drying must proceed with the paper free or sufficiently so, to practically assume its own dimensions, as in air drying, until another definite point near dryness, after which constraint again becomes unobjectionable.

During the commercial operation of a drying apparatus embodying this principle, the percentage of moisture content of the paper at the point of transfer from mechanically controlled to mechanically free drying, will unavoidably wander somewhat from the exact value sought; any such departure, if appreciable in amount, will have some detrimental effect on flatness if in one direction or strength if in the other. Care-

ful attendance, supplemented if necessary by one of the well-known devices for controlling the temperature of the drying rolls, will be sufficient to maintain an adherence 5 to best conditions sufficiently exact to insure great benefit; it will be readily understood, however, that a mere rough approximation to the optimum is not sufficient for best results. Further, the conditions 10 obtaining during air-drying are by no means a matter of indifference, and those found to be best are indicated in due course.

Our theory as to the explanation of the 15 various facts that we have discovered seems to us to further elucidate the matter, and to render more easy the practice of our invention, and the development of slight modifications within its scope; we therefore outline this theory, although it is to be carefully observed that the benefits and improvements that we have obtained can be fully 20 realized through the exercise of reasonable skill in following the directions herein set forth, without acceptance of, or regard to, 25 the correctness of our theory.

We conclude that the paper-making fibers, during the initial wet phase of mechanically constrained drying, move or slip upon each other so that they establish progressively 30 new mutual relations as the necessarily uneven drying goes on and as vapor is discharged from the wet mass, and that, so long as a very large percentage of water is present, this water and the hydrolyzed surface 35 of the fibers act as a lubricant, which, in conjunction with the mechanically loose fiber arrangement of the water-permeated sheet, allow such slippages to be continually occurring and mending themselves without bringing about new fiber relations inferior to the old as a starting point for the 40 progressive establishment of the mechanical and adhesive bond between the fibers when in due course the drying comes toward its final stages.

On the other hand, when drying has proceeded to a stage where there is no more water mechanically held by capillarity between the fibers, or wetting their surfaces, 50 then we conclude that further drying out of the water, more intimately absorbed or combined in the fibers themselves has a different result that explains the sudden change in effect of stretch or constraint. After this 55 point, further relative movement of the fibers can indeed take place, and the bond between them is permanently injured thereby, as in an incipient tear. This injury may be partly analogous to the injury to the adhesive bond between two glued surfaces 60 which results if movement takes place after a partial setting of the glue; also an incipient mechanical disentangling or de-felting action doubtless occurs, and a full re-establishment of mechanical intertwining is not

possible on account of the impaired freedom of motion of the fibers in the damp as compared with the wet sheet.

Further, our experiments appear to show that the beginning of the drying out of this 70 water of hydration (as it may be called in contrast to the mechanically held water) marks the beginning of the shrinkage of the paper at a definite rate proportional to the loss of moisture;—a fact which is believed 75 to indicate the establishment of a definite inter-fiber relation at this point, after which undue constraint or stretch will either permanently impair this relation, or possibly injure the component fibers themselves. 80

There has been hitherto some appreciation of the ill effects of excessive stretch of the drying web of paper, but, so far as we know, it has always been assumed that any such injury would grow progressively and 85 proportionately from the beginning of drying, as indicated by the dot-and-dash line in Figure 1. We believe that there has been no previous suggestion of the true condition disclosed by our experiments, 90 namely, the existence of a critical moisture value above which constraint did practically no harm and below which it seriously impaired strength.

If this increasing susceptibility to injury 95 by mechanical constraint actually did proceed regularly and corresponded in approximate quantitative proportion to the amount of water that had been removed, then increased value of the product due to the gain 100 in strength to be expected from any innovation in drying method that began tardily enough to be compatible with flatness, would not repay for necessary machinery and attendance; so that the mere qualitative, as 105 distinguished from quantitative, theory of this subject would not encourage action along these lines, and in fact has not encouraged it. Our experiments have disclosed the previously described wide departure 110 from direct proportionality between drying and susceptibility to injury, and the existence of the well marked critical point and range that place the commercial possibilities upon yet another footing. 115

As already stated, the point from which our experiments show that the paper must be allowed to dry with free shrinkage, if full strength is to be conserved, coincides substantially with the point at which it first 120 becomes dry enough to be immune from serious cockling under further drying without mechanical flattening. This result would be expected if our theory is correct, since we believe that this point marks the removal 125 of the last of the mechanically-held water, and the establishment of a fairly firm bond between the fibers such as would strongly oppose exactly that permanent change of fiber relation under locally uneven drying. 130

which is believed to subsequently produce cockling when the paper is fully dried.

Whether our explanation of the facts be correct or not, we have definitely established 5 the facts themselves to wit,—that the loss of strength from mechanical constraint in drying nearly all occurs within a rather short and very definite critical moisture range; that enforced flatness and tension 10 within the values usually employed do not appreciably detract from strength before this critical moisture range is reached in the process of drying; and that the beginning of this critical range is about coincident with the moisture content at which the 15 paper may begin substantially unconstrained drying without serious departure from ultimate flatness.

As a means of further elucidating this 20 matter, Figure 1 shows a mean graphical record of a number of experiments. On this plot ordinates show strength developed by the specimen which had been dried on the machine to, but not beyond, the percentage moisture content indicated by the 25 corresponding abscissa, and had been air-dried from that point on to dryness. In other words, the moisture content at which the drying was changed from constrained 30 to free, is plotted against the strength finally attained by the specimen, this strength being expressed as a percentage of the maximum strength the specimen would have attained had it been dried without constraint 35 from its point of delivery from the press rolls.

From this curve, which directly represents results on writing papers, it will be 40 seen that the critical point at which injury from constrained drying begins is relatively sharply defined, and that the range of moisture content, during which such drying is 45 detrimental, is in the general order of a fourth of the total range. So far as is known to us, the existence of any such critical point or critical range had not heretofore 50 been suspected by persons skilled in the practice of the art of drying paper, and even after its existence is known, there is 55 nothing in the behavior of the paper during or after passage through the machine from which a skilled man would be able to deduce or infer its existence, and still less, its location; for this reason it will be necessary for 60 persons practicing this invention to ascertain by performance of, or reference to, actual experiments, the critical moisture percentage and moisture range for the particular kind of paper that it is proposed to dry, and not to depend upon mere skill in the 65 paper drying art in determining the range through which the drying paper should be freed from strong mechanical constraint. It will be understood that the quantitative results would be quite different in widely dif-

ferent papers, such as papers made from a slow stock as contrasted with those made from a free stock.

By way of a specific illustration we here-with give the mean numerical results from 70 five series of experiments showing injury from drying various weights of a certain fairly high grade writing paper by the customary method; the paper came from the press-rolls to the ordinary paper machine 75 drier with moisture content equal to a little over 200% of the weight of the dry fiber. The drying operation did not measurably injure the strength up to the point where the contained moisture has been reduced 80 from this initial value of 200% down to 61% of the dry weight of the paper; the further reduction of the moisture content from 61% to 5% of the dry weight resulted in a reduction of Mullen strength by 24.0% 85 of the maximum strength possible, or otherwise stated by 31.6% of the final strength actually realized and the further reduction of the moisture from 5% to practical dryness did not further injure the strength appreciably. The same data are otherwise presented in Figure 1. Expressing approximately the same results in terms of the moisture content of the paper as it reaches the 90 drier, it may be said that the drying under 95 severe mechanical constraint should cease when the moisture content of the paper has been reduced to 25% to 50% of total weight of the moist paper. In other words, for all practical purposes, the critical point, at 100 which the further drying of such paper should be without considerable mechanical constraint, lies within a range of 25% to 50% of the moisture content depending to some extent on the stock undergoing treatment, and usually lies within a range of 105 35% to 45%.

From this discovery it has been possible to work out important improvements in 110 drying and the process and apparatus that we have found most advantageous will next be described with reference to the drawings. The operating details of the process, and the proportions of the apparatus will require 115 suitable changes to meet variation in kind of paper dried; such of these changes as are not directly indicated can be readily worked out by persons skilled in the art and conversant with this disclosure. The arrangement here described is one directly 120 adapted to writing papers.

In our process the paper in a continuous traveling web is taken from the wet end of the Fourdrinier or other web-forming machine end dried to the first critical point 125 previously defined, under such mechanical constraint as will forcibly determine flatness; it is then passed to an apparatus in which the drying is continued with the paper, free or sufficiently so to take up its 130

own form and dimensions, and the drying is here continued at least through that phase susceptible to injury by strong stretch or mechanical restraint. The drying may be 5 carried on to completion with the paper still unconstrained, but we should not regard it as a departure from our process if the paper were transferred back to apparatus where flatness is enforced, as soon as the phase 10 susceptible to injury by constraint is passed.

Reference may be had to the drawings, which show an apparatus well adapted to carry out this process:

Figure 1 represents the chart previously 15 referred to; Figures 2 and 2<sup>a</sup> show a side elevation of the apparatus, and Figure 3 a plan of the part in which the second or unconstrained phase of the drying is carried on.

For the first phase of drying, we prefer 20 to use the ordinary "dry part" of the usual paper machine, as illustrated in Figure 2; but modifications of, or departures from, this structure, such as the so-called "Yankee" drier, or a drier where some slatted 25 rolls are substituted for part of the solid ones, are permissible if they still provide for adequately holding the paper flat during this phase of the drying.

The second phase of the drying may be 30 satisfactorily carried out in the well known festoon drier, such as that illustrated or by any other drier which effects drying of the paper without severe constraint. There are certain important operating details that 35 should be kept in mind in the proportioning and handling of this form of drier for this purpose, and these are indicated later. Any equivalent form of drier may be substituted for the festoon drier in this second phase,— 40 equivalence for this purpose meaning similar ability to remove moisture evenly from the paper while it passes through the drier in a condition comparatively free from mechanical stress or constraint.

The third comparatively brief phase of 45 drying, after the paper has become so dry as to have recovered immunity from injury through ordinary degrees of mechanical constraint, can, if desired, be carried out on drying cylinders similar to those of an ordinary paper machine, since the action of the felts, and the tension, promote flatness and finish desired by the trade for most papers.

On the drawing, we have indicated at A 55 the delivery end of a Fourdrinier machine, for which any other web-forming machine may be substituted, by which the initially wet web of paper is newly formed and at B we have indicated a plurality of the usual 60 press rolls which may be of standard form. At C we have shown a standard drier employing drier felts, to which the web is delivered from the Fourdrinier machine and the press rolls, and by which the web is 65 under tension and constraint, as usual to

predetermined form and dimensions, during its initial drying, in accordance with our process. This drier is shown as having but the first twelve heated rolls, (out of the usual twenty-three or more) the temperature of 70 which is controlled as ordinarily. The number of heated rolls will naturally vary with their speed and the temperature and with the character of the paper being dried. At

75 D we have shown conventionally an apparatus in which the drying of the paper may be continued, after it has reached the critical point of moisture content, beyond which

severe mechanical constraint would tend to injure the ultimate product. This apparatus 80 is used during the second phase of the drying and as shown it may include a closed casing in which the paper is festooned by any suitable festooning mechanism. This

particular apparatus per se forms no essential 85 feature of the present invention and is not claimed herein. The air is drawn into the apparatus through a conditioning instrumentality 5 by which it is charged with a definite degree of moisture; thence, 90 through suitable dampers, the air passes into a heater 6 by which it is heated to a suitable temperature and from which it is delivered to a manifold 7 at the top of the delivery

95 end of the apparatus and directed downwardly between the folds of paper on the festooning mechanism. A damper is indicated at 8, by which a portion of the moisture-laden air may be drawn from the drying enclosure at the bottom of the apparatus, and be redelivered to the heater 6. 11 represents a fan which is employed for ensuring the circulation of the air. At the forward or receiving portion of the apparatus, there is a second top manifold 12 to which the air

100 withdrawn through a conduit 13 leading from the manifold 9 may be supplied by a conduit 14 and a fan 15. In the conduit 14 there is arranged a heater 16 into which additional outside air may be supplied by a 105 damper 19 and air from the apparatus may be supplied through a damper controlled conduit 23. From a manifold 20 at the bottom of the first portion of the apparatus, the air is withdrawn by a fan 21 and discharged

110 through a conduit 22. The drying of the paper may be completed in this apparatus, although for some purposes it may be desirable to again subject the paper to drying 115 under restraint, and consequently we have shown at E several rolls of the usual standard drier equipped with the drying felts. As we have already stated, it is not at all necessary in the second phase of drying to

120 employ a festooning apparatus, as we may employ in lieu thereof any other form of drier in which the paper is substantially free from undue mechanical constraint or tension and is free to substantially assume its 125 own form and dimensions, as the paper dur-

ing this second phase of the drying may be freed from constraint without danger of cockling.

With regard to the proportions and adjustments of the apparatus, the following may be said:

The earlier part of the drying, which is carried out on ordinary paper-machine dryers, will present only one unusual difficulty to persons skilled respectively in the arts of paper-machine designing and paper-machine operation; namely, the substitution of the requirement that the percentage of moisture in the paper at the end of this section be held within relatively narrow definite limits, for the less severe customary requirement that the paper emerge with any moisture content less than a specified small amount. It is well known that the discharge of moisture from the wet paper as it passes over the successive drying drums or cylinders of the paper-machine drier is at first rather slow; that after the paper and its contained water is heated to nearly the boiling point by contact with the earlier hot drums this rate of discharge becomes materially greater; and that when drying is nearly complete it becomes much less again because there is little moisture left to evaporate; so it will be understood that the fact that this first section removes say, 70% of the amount of moisture that the paper initially contained does not imply that just 70% as many drums should be used as in a complete drier of usual form. As an example of this, experiments with certain writing papers showed in that particular case the best results were obtained with a first section having the first 12 rolls, of a 23-roll machine.

The proportions of this first-phase drier having once been fixed, working adjustment can be obtained by variation of steam pressure and consequent temperature of the drying steam in the drums, by variation in the speed of the drums and in some measure, by control of the pressure of the press-rolls. It will be understood that to secure the best results the operation must be controlled carefully, since an exact end point is sought at a phase of the drying where the discharge of moisture is rapid; while in ordinary practice an approximate end point is permissible, and the final phase is one where the moisture discharge is slow.

In the second part of the drying where the paper is free from any strong mechanical constraint, a suitable (but not the only) method of carrying off the contained moisture is by means of a current of air, as in the festoon drier illustrated. In using such a method it is desirable that the location of delivery, the temperature, volume, and humidity of the air serving this function be so regulated that the edges will not dry before the middle of the web, nor the outside of

the sheet too much faster than the inside. It is of course also highly desirable that the rate of drying should be as high as may be compatible with these conditions. The end point for the unconstrained drying need not be so precisely maintained as in the case of the first part, since for substantially optimum results it is only necessary that the paper emerging from this second section contain no more than a definite amount of moisture—not that it contain exactly that amount. Indeed, as already stated, a good commercial result is still obtained if the drying is carried to completion in this section.

The third section in which the paper is carried to substantial dryness may, if desired, well be of the standard form, as illustrated in Figure 2, and its design and its operation will present no unusual difficulties to those skilled in these respective arts. Of course if the paper is thereafter subject to some after-process that wets it, as top sizing, it must be dried again, but our process is directly concerned with only the initial drying.

Paper dried in a continuous web in a machine of the character just disclosed differs from that dried in the usual way, wholly under constraint, principally in the possession of materially higher strength; there are also certain other differences in the matter of texture, feel and finish, all of which, so far as we are aware, further contribute to conferring upon the product a higher degree of utility and value than it would have possessed had the drying process and apparatus been of standard character.

This sequence of drying operations as herein disclosed, must start with the newly-formed wet sheet, and be carried on continuously, in order to produce the most valuable results; that is, the paper must not have been dried before and afterward wetted again; and it should not be partially dried under constraint, rolled up, and subsequently or elsewhere transferred for further drying to an apparatus exerting no strong constraint. The reason for the first limitation is that if the natural bond between the fibers is once weakened by detrimental drying methods such as universally heretofore practiced, the injury cannot be repaired by any after-treatment. The reason for the second limitation is that paper, so wet as is that at the point of transfer, cannot by any known feasible process or system be rolled up, stored, transported and re-handled without such serious injury and loss as would more than offset the benefits of the process.

Paper dried in accordance with our process may undergo immediate or deferred after-treatment such as tub-sizing, and it will maintain the increased strength and improvement in texture without impairment by such after-treatment, and in the case of

tub-sizing, will derive as much additional benefit in the matter of added strength from the top-size as it would have done had it gone to this treatment weakened by detrimental drying.

It is therefore to be clearly understood that our process is one for conserving the natural maximum strength of the paper and preventing injury or detriment thereto during the process of drying; and is not a process for conferring additional strength by any after-treatment to be administered to a web or sheet that has already been once dried, or of so administering any such after-treatment as to maximize the additional strength so conferred. Our product is susceptible equally with the product of methods heretofore used, of modification by, or benefit from such after-treatments, however administered. Its very substantial inherent advantages over the product of drying methods heretofore standard, is due to the removal by our process of a source of injury which has hitherto been present—not to the addition or manipulation of any agent or treatment adapted to confer desirable qualities after the paper has once been injured during its first drying.

Having thus explained the nature of our invention and the principles of the necessary operation of instrumentalities employed in connection with the process, but without attempting to set forth all of the various instrumentalities which might conveniently be used since we make no claim to any instrumentality per se, what we claim is:

1. The herein described method of drying paper, which consists in progressively removing from the initially wet newly formed paper, as it is delivered from the web-forming machine and while under mechanical restraint, a portion of its contained moisture to a point at which flatness of the ultimate product is secured and beyond which injury to the strength of the ultimate product would result, and then drying the paper while substantially free from severe mechanical constraint.

2. A process of drying paper, which consists first in progressively drying an initially wet newly formed traveling web of paper, while mechanically constrained to substantially determinate form until the moisture content is reduced to a point beyond which further constraint would cause injury to the strength of the ultimate product, and, second, in further progressively drying such paper without substantial mechanical constraint.

3. The following process for drying paper, to wit: first, subjecting an initially wet newly formed traveling web of paper to progressive drying, while being forcibly held to substantially determinate form and dimensions, until the moisture content is reduced to a first critical value marking the beginning of injury from such mechanical constraint; second, immediately and continuously subjecting the same to further progressive drying without any considerable degree of such constraint, until the moisture content has been further reduced to a second value at which immunity from injury by customary degrees of mechanical restraint is reestablished; and, third, completely drying the web while under constraint.

4. A process of drying paper which consists in drying the newly formed web of paper down to a certain critical moisture content under such relatively strong mechanical constraint as will forcibly determine flatness, and immediately thereafter further drying it at least down to a second critical moisture content, without any considerable constraint; the two critical moisture values being defined as boundaries of a critical moisture region throughout which the progressively drying web of wet or damp paper suffers important injury to strength from any strong constraint, and outside of which it suffers no such injury therefrom.

5. A process of drying paper which consists in causing a traveling newly formed initially wet web of paper to be passed under tension through the heated rolls of a suitable drier until a point is reached beyond which injury to the strength of the ultimate product would result, and then removing tension from the web and further drying the same until the desired point of moisture content is reached.

6. The herein described process of drying writing paper, which consists in first subjecting a traveling newly-formed web of initially wet paper to progressive drying, while being mechanically constrained to substantially definite form, until the moisture content is reduced to a point lying between 25% to 45% of the total weight, and then progressively further drying such partially dry web free from any considerable degree of mechanical constraint.

In testimony whereof we have affixed our signatures.

EMIL A. BRINER.  
HENRY J. GUILD.